

H. AITKEN.  
TREATING IRON ORE, &c.

No. 82,576.

Patented Sept. 29, 1868.



# United States Patent Office.

HENRY AITKEN, OF FALKIRK, SCOTLAND.

*Letters Patent No. 82,576, dated September 29, 1868.*

## IMPROVEMENT IN TREATING IRON-ORES, &c.

The Schedule referred to in these Letters Patent and making part of the same.

TO ALL WHOM IT MAY CONCERN:

Be it known that I, HENRY AITKEN, of Falkirk, Stirling county, Scotland, have invented an Improvement in Treating Iron-Ores, &c.; and I do hereby declare the following to be a full, clear, and exact description of the same.

My invention consists in subjecting iron-ores and iron-stone, during the process of coking, to the treatment fully described hereafter, so as to utilize the volatile portions of the material, and obtain a better and more available product at less expense than by the ordinary processes.

In order to enable others skilled in the art to practise my invention, I will now proceed to describe the manner of carrying it into effect, reference being had to the accompanying drawing, which forms a part of this specification, and in which—

Figure 1 is a sectional elevation of one form of apparatus which may be employed in carrying out my invention.

Figure 2, a section on the line 1-2, fig. 1; and

Figure 3 a plan view of part of the apparatus.

A is a platform, upon which the iron-ores or iron-stones are placed, and B perforations, through which the heat and products of combustion are drawn downward into the flues C, through which they pass to the condensing-pipes D, by means of the action of the steam-jet issuing through the nozzle H, these pipes D being connected with suitable vessels, wherein the condensable matters are collected and preserved for use.

E is an iron arched covering, the inside of which may be lined with fire-bricks, or other suitable materials, as shown in figs. 1 and 2. The arched covering E is carried upon wheels or rollers a, fig. 1, and shown dotted on fig. 2, so that, when the heap or layers of iron-ores or iron-stones are built or laid upon the platform A, it is covered by the arched covering E, which is run along the rails b, fixed on the side walls F. By this means, any convenient size of heap may be formed, as the arched covering is, by preference, made in sections, and each of which is run along the rails b, and placed close to each other, until the heap is covered.

The iron-ores or iron-stones may be fired or ignited on the top, and the cover E run over the heap, the heat or gases being drawn down, as above and hereinafter described.

To prevent danger from explosions, or a high pressure of gas, which may occur during the carbonizing of the iron-ores or iron-stones, part of the end, G, which encloses the arched covering E, is hinged, as shown at c, fig. 2, so that it may be blown open, and the explosive or high-pressure gases may escape before they have collected to a dangerous extent.

Holes D are formed in the arched covering E, to admit air to the heap after it is fired.

To facilitate the condensing and collecting of the condensable matters during the carbonizing of the iron-ores or iron-stones, water may be caused to flow through the flues C and the pipes D. Steam and water may be also injected among the iron-ores or iron-stones, from time to time, while combustion is going on, to facilitate the condensation of the gases, and, towards the end of the process, steam and water may again be admitted, for the purpose of facilitating the separation of the sulphur and salt, or salt water may be admitted to render what sulphur remains harmless. The gases which are not condensed escape by pipe D to a chimney or fire-grate, not shown in the drawings, or the exhausting of the gases is maintained by any exhausting or forcing-apparatus or means.

When the coking or carbonizing-process is finished, the arched covering may be run off on the rails b, and the iron-ores or iron-stones may be removed, or reduced at once to malleable iron, steel, or pig-iron, or the cover may be kept on, and the iron-ores or iron-stones may be cooled, and watered out under it, and then removed, after which they may be reduced by the blast-furnace into pig-iron, or they may be reduced into pig-iron, steel, or malleable iron, in kilns, ovens, or air-furnaces.

In lieu of using a steam-jet or chimney for exhausting the gaseous matter, as hereinbefore set forth, a jet of air at high pressure may be employed, by connecting the nozzle with a reservoir in which the air is com-

pressed. This air in expanding, on escaping through the nozzle, will reduce the temperature of the condenser to the requisite degree, at the same time producing the necessary amount of draught.

I may further explain that when carbonizing iron-ores or iron-stones, which are not rich in carbonaceous matter, to facilitate and quicken, the time for carbonizing them, a portion of other carbonaceous or hydrocarbonaceous matter, such as coal, dross, or oil may be mixed with the charge, and the two being treated together, besides diminishing the period of carbonization, produce a carbonized material, which, containing a larger proportion of carbonaceous matter than is naturally combined with it, less fuel for after reduction is requisite.

In the cases of iron-ores or iron-stones which become soft or friable by carbonization, the mass may be hardened by pouring crude hydrocarbon-oil or tar over it when at a high heat.

The materials to be carbonized may be placed on a frame or platform carried upon wheels, or on revolving plates or platforms, such platforms or plates being arranged to traverse on rails or trams, that they may be run under an arched covering or kiln, and therein coked or carbonized, or the process may be made continuous by feeding the raw iron-ore or iron-stone in at one end of the kiln, retort, oven, or arched covering, and, as it is coked or carbonized, drawing it out at the opposite end, the gases and oils being utilized or collected as hereinbefore described.

I claim as my invention, and desire to secure by Letters Patent—

1. Coking iron-stone or iron-ore upon a perforated platform, through the openings in which, and through the mass of stone or ore, the gaseous products of the coking-operation are drawn downward, for the purpose described.

2. Utilizing the gaseous products of the coking of iron-stone or ore, substantially as specified.

3. The coking or carbonizing of iron-ores or iron-stones, in combination with carbonaceous or hydrocarbonaceous matter.

4. The employment of crude oil or tar, or oily or tarry matter, for hardening coked or carbonized iron-ores or iron-stones.

In testimony whereof, I have signed my name to this specification in presence of the two subscribing witnesses.

HENRY AITKEN.

Witnesses:

ST. JOHN VINEMDAZ,  
JOHN BROWN.